

Jan. 1, 1952

N. E. WIDELL

2,580,984

CORROSION INHIBITOR IN ABSORPTION REFRIGERATION SYSTEM

Original Filed Feb. 8, 1946



INVENTOR.  
Nils Eric Widell  
BY  
Howard A. Venard  
his ATTORNEY

## UNITED STATES PATENT OFFICE

2,580,984

CORROSION INHIBITOR IN ABSORPTION  
REFRIGERATION SYSTEMNils Erik Widell, Stockholm, Sweden, assignor to  
Aktiebolaget Elektrolux, Stockholm, Sweden, a  
corporation of SwedenOriginal application February 8, 1946, Serial No.  
646,394. Divided and this application May 12,  
1951, Serial No. 225,934. In Sweden January  
22, 1945

2 Claims. (Cl. 62—179)

1

This invention relates to absorption refrigerating apparatus and more particularly to such apparatus of the inert gas type wherein the absorption solution contains a corrosion protective substance. This application is a division of my application Serial No. 646,394, filed February 8, 1946.

The main object of the invention is to increase the lifetime of the apparatus and to prolong the durability of the corrosion protection. The invention is of particular importance in such refrigerating apparatus wherein absorption solution from its normal circulating system through the boiler and absorber of the apparatus is brought into contact with working medium having a higher refrigerant concentration than that of the absorption solution.

The invention will be hereinafter more fully described with reference to the accompanying drawing showing diagrammatically an embodiment of the arrangement according to same and in this connection further characteristic features of the invention will be set forth.

The figure shows diagrammatically an absorption refrigerating apparatus, wherein water is used as an absorbent and ammonia as refrigerant. Referring to the figure reference numeral 10 denotes a tube acting as a flue, to which heat is continuously supplied from a heat source, not shown, for example an electric cartridge, a gas or petroleum burner. The boiler of the apparatus is designated by 11 and its liquid circulating pump by 12. The boiler pipe 11 is extended upwardly and at the top connected to the air cooled condenser 13 of the apparatus. Further numeral 14 denotes a so-called pressure equalizing vessel of a kind known per se which through a drainage conduit 15 communicates with the evaporator of the apparatus designated by 16. In said conduit 15 the condenser pipe 13 opens, from which liquid refrigerant thus flows by gravity to the evaporator through the conduit 15. Further numeral 17 designates the gas heat exchanger of the apparatus and 18 its air-cooled absorber. Numeral 19 indicates a vent conduit through which the pressure equalizing vessel 14 freely communicates with the gas circulating system of the apparatus. Said system is formed in a way known per se as is the liquid circulating system of the apparatus. The enriched solution in the absorber vessel 20 of the apparatus thus streams through its liquid heat exchanger 21 and the main pump 12 to the boiler 11 and thence it returns through the heat exchanger 21 and a conduit 22 to the absorber 18.

In accordance with usual practice the appa-

2

ratus is formed of iron pipes joined together by gas welding. Before filling the apparatus it is evacuated of all air, and as ammonia by itself has no influence upon iron in absence of oxygen, no corrosion should be feared in the internal iron walls. However, these walls formed of ferrous metal will nevertheless be affected by the ammonia solution by the forming of complicated iron compounds, by which the walls after a relatively short time would be loosened up and lose their strength against the high pressure (about 20 atm.) prevailing in the apparatus. In order to avoid such corrosion an alkali salt of sodium chromate ( $Na_2CrO_4$ ) has previously been dissolved in the absorption solution. The chromatic concentration required in the absorption solution for counteracting the corrosion is extremely small and may be counted in fractions of per cent. However, the chromate is slowly consumed and therefore it has previously been necessary to utilize a concentration of chromate in the solution many times higher for the purpose of creating a chromatic reserve, covering several years' consumption. Salts dissolved in the absorption solution will, however, influence the pumping in the thermosiphon pump 12 in an unfavourable direction and therefore until now it has been necessary to limit the concentration of chromate in the solution to a concentration corresponding to about 2% of  $CrO_4$ .

In different ways, however, it has been attempted to form an additional reserve of alkali chromate by enclosing in the absorber vessel a storage of solid sodium chromate in a container with a limited communication with the surrounding solution, whereby a gradual dissolving of the solid chromate has been attained. It has not been possible to make the dissolving so uniform that the concentration of the solution with security can be kept below the values wanted. The velocity of dissolving has also appeared to be dependent upon a plurality of uncontrollable factors, among other things the operating temperature which very essentially varies with the climatic condition under which the apparatus is operated. According to this invention a reserve of chromate of an arbitrary greatness may be arranged in the apparatus. The invention is substantially characterized thereby that the absorption solution of the apparatus is saturated with a salt of the chromatic acid, having a solubility in said solution not exceeding 2%. Further, the solubility of the present chromate may be as much as possible independent of the temperature, though certain variations with the temperature

may be permitted. A particularly suitable chromate is strontium chromate ( $\text{SrCrO}_4$ ). The solubility of strontium chromate in the absorption solution is so small that the saturated solution only contains 0.01 to 0.2% of  $\text{CrO}_3$ .

Apparently this small quantity of chromate which originally, when filling the apparatus, is dissolved in the absorption solution will be comparatively rapidly consumed. It is therefore generally necessary to enclose a reserve of solid strontium chromate in the apparatus. According to the invention therefore a container 50 is arranged in the absorber vessel 20 or possibly in another vessel interconnected with the liquid circulating system of the apparatus. The reservoir 50 may suitably include a short piece of pipe, both openings of which are covered with a fine-meshed iron net and in which a pressed tablet of strontium chromate is inserted. The container may suitably be attached to the wall of the vessel by a strip or similar member which is attached to the wall of the vessel and to the wall of the container 50 by welding. The support is denoted by 51. When the liquid contents of the absorber vessel 20 is continuously renewed, the absorption solution will automatically become saturated gradually as its contents of chromate decreases during its passage through the absorber vessel 20. The pressing of the solid strontium chromate into a tablet possesses the advantage that no solid particles by mechanical influence of the streaming solution will follow the liquid through the narrow passages of the apparatus. In order to improve the strength of the tablet small amounts of sodium hydroxide may be mixed with the chromate when pressing said tablet.

As already mentioned, the invention is of particular importance in such absorption refrigerating apparatus in which the absorption solution is now and then brought into contact with liquid refrigerant, the concentration of which thus attains high values. This is the case in the absorption refrigerating apparatus shown in the figure. From the lower part of the boiler pipe a conduit 23 runs out, which opens into the pressure equalizing vessel 14 and forms an auxiliary pump for raising the absorption solution to said vessel. Thence, the warm solution streams through the conduit 15 into the evaporator coil 16 and thence through the exchanger 17 and the absorber 18 to the absorber vessel 20. In contradistinction to the main pump 12 the auxiliary pump 23 is not immediately heat conductively connected with the flue 10 but instead arranged in heat conductive relation with a hermetically closed heat transfer system which is welded to the flue 10 along a welded seam 42. The system contains a heat transfer medium with a high boiling point, possibly in addition to an auxiliary medium with a lower boiling point. The transfer medium is vaporized in the boiling part 41 of the system and condenses to liquid in a container 30 where the condensate is accumulated. Some part of the vapours, however, give off their heat contents to the pump pipe 23. After a certain period the system is boiled dry, and all the condensate remains stor-

aged in the container 30. This container is connected by a flexible member 31 with the system, thus permitting it to be raised for tilting the liquid contents. In this way a method of controlling the heat transfer system is attained, thus causing the pump 23 to operate whenever desired and after a certain period automatically to stop working. The solution raised by the auxiliary pump 23 streams in the way already described into the evaporator where it, however, is mixed with refrigerant condensate entering from the condenser 13, having an ammonia concentration from 80 to 100%. The supply of condensate from the condenser 13 takes place continuously. This supply of absorption solution to the evaporator 16 has for its object, when required, to effect melting of ice formed thereon. It has appeared that a solution of sodium chromate of 1 to 2 per cent cannot be mixed with ammonia having the concentration existing in the evaporator without most of the salt being precipitated into solid form. The salt precipitated would collect in the evaporator and would very soon effect a blocking action and at the same time such precipitated salt for the future would be prevented from taking part of the corrosion protection. A solution of strontium chromate remains, even if it is saturated, approximately unaffected by an increase of the ammonia concentration and the small amounts of chromate which possibly may be precipitated will be replaced from the reverse 50 provided in the absorber vessel.

Though the strontium chromate is very little soluble in the absorption solution, that is, in the ammonia water mixture, the concentration of protecting substance in this chemical compound is sufficient to effect a satisfying corrosion protection.

What is claimed is:

1. In the art of refrigeration employing an absorption refrigeration system formed of ferrous metal and utilizing ammonia as refrigerant and water as an absorbent, that improvement which comprises maintaining in the aqueous ammonia solution a supply of solid strontium chromate.

2. In the art of refrigeration employing an absorption refrigeration system formed of ferrous metal and utilizing ammonia as refrigerant and water as an absorbent, that improvement which comprises maintaining in the aqueous ammonia solution a solid body of matter including strontium chromate and sodium hydroxide mixed therewith.

NILS ERIK WIDELL.

#### REFERENCES CITED

The following references are of record in the file of this patent:

#### UNITED STATES PATENTS

| Number    | Name       | Date          |
|-----------|------------|---------------|
| 1,960,040 | Widell     | May 22, 1934  |
| 2,210,611 | Widell     | Aug. 6, 1940  |
| 2,246,665 | Buffington | June 24, 1941 |
| 2,402,413 | Kagel      | June 18, 1946 |
| 2,457,334 | Widell     | Dec. 28, 1946 |